# EUROPEAN PATENT SPECIFICATION

(11) **EP 1 968 795 B1**
(45) Date of publication and mention of the grant of the patent: **22.02.2012**
(21) Application number: 06828036.1
(22) Date of filing: 19.12.2006
(51) Int. Cl.: B41N 1/04

(54) **MANUFACTURE OF PRINTING CYLINDERS**
HERSTELLUNG VON DRUCKZYLINDERN
FABRICATION DE CYLINDRES D'IMPRESSION

(30) Priority: 23.12.2005 AU 2005907288
(43) Date of publication of application: 17.09.2008
(73) Proprietor: Commonwealth Scientific and Industrial Research Organisation, Campbell, ACT 2612 (AU)
(72) Inventor: ZAHIRI, Saden, Mt Waverley, Victoria 3149 (AU); JAHEDI, Mahnaz, Toorak, Victoria 3142 (AU); ANTONIO, Christian, Tarneit, Victoria 3029 (AU)
(74) Representative: Barnfather, Karl Jon
(86) International application number: PCT/AU2006/001930
(87) International publication number: WO 2007/070939

(56) References cited:
- EP-A- 0 623 466
- EP-B1- 0 902 100
- WO-A1-00/06393
- WO-A1-94/26534
- US-A1- 2003 138 570
- US-A1- 2005 153 821

## Description

The present invention relates to a method for the manufacture of cylinders (rollers) for the printing industry. More specifically, the present invention relates to the manufacture of cylinders for use in gravure printing processes. The present invention also relates to printing cylinders, including gravure printing cylinders, that have been manufactured in accordance with the method of the present invention.

In gravure printing processes an image is etched on to the surface of a metal plate to produce a recessed image, the recessed image areas are filled with (rapid-drying) ink and the plate rotated in contact with a substrate upon which the image is to be presented. The surface of the cylinder must have certain characteristics that render it suitable for use in the printing process. Thus, the surface must be capable of being engraved with an image, and this is normally done by chemical etching or electromechanical engraving. The surface must also have a good quality (mirror) finish to provide high quality printed images and be hard wearing so that the cylinder has a suitably long working life without deterioration in print image quality.

Conventionally, the cylinders used in gravure printing comprise a steel or aluminium substrate cylinder coated with a layer of copper into which an image may be engraved. Typically the copper layer is provided on the substrate cylinder by electroplating. This can be a relatively slow process, especially as the substrate cylinder needs to be pre-prepared before electroplating can be commenced because copper does not adhere well to steel or aluminium when applied by electroplating. Thus, prior to electroplating, it is conventional to apply a layer of copper cyanide to steel and a layer of zinc and then a layer of nickel to aluminium. Electroplating also tends to consume a lot of water and electricity and involves the use of chemicals that are not environmentally friendly.

In practice, the electroplated copper layer does not have very good wear characteristics and it is therefore also conventional to apply a layer of chrome over the top of it. This is also normally done by electroplating and therefore has the associated drawbacks mentioned above. In the finished cylinder the image is engraved in the copper layer and then a very thin layer of chrome is deposited on the engraved copper surface. Thus, the copper carries the image and the chrome protects it.

Against this background, it would be desirable to provide a process for manufacturing a printing cylinder that does not rely on electroplating technology and that does not suffer the drawbacks described. Specifically, it would be desirable to provide a printing cylinder by a method that is simple to implement and that has relatively high throughput, that does not require pre-preparation of a substrate cylinder, and that produces a print surface that has desirable wear characteristics.

US 2005/0153821 relates to a method of manufacturing a metal surface, for the purpose of creating a substrate suitable for coating, about a cylindrical core such as a fluid metering roll or fluid metering sleeve, comprised of carbon fiber composite, glass fiber composite, Kevlar fiber composite, other composite, foam, rubber, polymer, plastic, or any combination thereof. The method involves wrapping the cylindrical core with wire composed of aluminum, nickel, steel, stainless steel, or other metals or alloys thereof that may be formed into a wire and applying coatings of metal, ceramic or carbide or combinations thereof.

Accordingly, the present invention provides a method of manufacturing a printing cylinder, which comprises cold-gas dynamic spraying of metal or metal alloy particles directly onto a substrate cylinder. More specifically, the method of the present invention involves cold-gas dynamic spraying of metal particles or metal alloy particles of a predetermined composition onto a steel, aluminium or polymeric composite substrate cylinder in order to provide a printing layer having suitable surface characteristics (capable of being engraved by conventional means such as electronic or laser, high hardness and excellent wear characteristics).

Cold-gas dynamic spraying (or cold spraying) is a known process for applying coatings to surfaces. In general terms the process involves feeding (metallic and/or non-metallic) particles into a high pressure gas flow stream which is then passed through a converging/diverging nozzle that causes the gas stream to be accelerated to supersonic velocities. The particles are then directed on to a surface to be coated. The process is carried out at relatively low temperatures, below the melting point of the particles and the substrate to be coated, with a coating being formed as a result of particle impingement on the substrate surface. The fact that the process takes place at relatively low temperature allows thermodynamic, thermal and/or chemical effects on the surface being coated and the particles making up the coating to be reduced or avoided. This means that the original structure and properties of the particles can be preserved without phase transformations etc. that might otherwise be associated with high temperature coating processes such as plasma, HVOF, arc, gas-flame spraying or other thermal spraying processes. The underlying principles, apparatus and methodology of cold-gas dynamic spraying are described, for example, in US 5,302,414.

Herein the expression "printing surface" means the (outer) surface of a printing cylinder that is capable of being engraved to provide a recessed image for use in a (gravure) printing process. In accordance with the present invention, and as will be described, it has been found possible to provide a printing surface on a cylinder substrate as a single, coherent layer having suitable surface characteristics.

In accordance with the present invention it has been found possible to produce a very dense (non-porous) printing surface on a cylinder substrate by suitable choice of the characteristics of particles to be sprayed (type and particle size distribution) and cold spray operating parameters.

An important aspect of the present invention resides in the composition of particles that are applied by the cold spray process. Thus, in one embodiment it has been found advantageous to apply by cold spraying particles of an alloy of copper and zinc. In this embodiment the composition of the powder to be sprayed is typically 88-99 wt% copper and 12-1 wt% zinc. Preferably, the composition comprises 91 wt% copper and 9 wt% zinc.

In this embodiment the average particle size of the individual components is likely to influence the density of the resultant coating. Preferably, the coating is dense and free from defects, micro-voids, and the like, since the presence of such can be detrimental to the quality of the engraving process and hence the printing surface of the cylinder. In the embodiment described, the average particle size is typically from about 15 to about 32 µm with average particle size of about 24 µm. One skilled in the art will be able to determine the optimum particle size or particle size distribution to use based on the morphology and characteristics of the layer that is formed by cold spraying. Metal particles suitable for use in the present invention are commercially available.

In this embodiment the thickness of the deposited layer is typically 300-350 µm. This will typically be reduced by machining to provide a final surface having a thickness of 150-200 µm.

In another embodiment of the invention the printing surface is formed by spraying particles of copper or an alloy of copper and zinc for electronic engraving, and with particles of zinc for laser or electronic engraving. As explained above, the particle size of the metallic particles used for cold spraying will influence the density of the resultant coating, with formation of a consolidated, dense, defect-free coating being desired. In this embodiment, the copper particles will typically have an average particle size of about 10 µm, for example 9 µm, and the zinc particles will have an average particle size of about 10 µm, for example 7 µm. The alloy particles will typically have an average particle size of from about 15 to about 32 µm. Particles useful in this embodiment are commercially available.

In this latter embodiment, the deposited thickness of the copper layer is typically 300-350 µm with the final (machined) thickness typically being 150-200 µm. The thickness of the deposited zinc layer is typically 250-300 µm with the final (machined) thickness being 150-200 µm.

Typically, the printing surface should have a Vickers hardness (VHN) of 225-240 kg/mm². However, copper printing surfaces formed in accordance with the present invention may not exhibit a suitable surface hardness. In an embodiment of the present invention it has been found that suitable hardness values may be achieved by methodology in which metallic particles as described are simultaneously deposited and heat treated through the cold spray process. This was accomplished by manipulating the temperature of the gas stream used in the cold spray process, the rotation speed of the substrate roller during deposition and the speed of the movement of the spray head. All the parameters are adjusted in a way to control the density of dislocations to give the desired hardness.

The substrate cylinders to which the printing surface is applied in accordance with the present invention are of conventional design and dimensions. The cylinder will be formed of steel, aluminium or a polymeric composite. Deposition takes place by positioning the surface of the cylinder adjacent the nozzle from which the metal particles will be accelerated. The distance between the end of the nozzle and the substrate surface (the stand off) may be varied to achieve a coating layer having the desired properties. The cylinder and nozzle will be moved relative to each other in order to coat the outer surface of the cylinder. Thus, the cylinder may be rotated about its longitudinal axis relative to the nozzle and the nozzle moved along the longitudinal axis of the cylinder. The speed with which the cylinder rotates and the nozzle moves along the longitudinal axis will influence the mechanical properties and the thickness of the printing surface that is deposited. The cylinders may be of a form that is otherwise used in the kind of electroplating processes described above.

The operating parameters for the cold spray process may be manipulated in order to achieve a coating that has desirable characteristics (density, surface finish etc). Thus, parameters such as temperature, pressure, stand off (distance between nozzle and substrate surface), powder feed rate and cylinder rotating speed may be adjusted.

The apparatus used for the cold spray process is likely to be of conventional form, and such equipment is commercially available. In general terms the basis of the apparatus used for cold spraying will be as described and illustrated in US 5,302,414.

After manufacture in accordance with the present invention the printing roller are typically machined and polished (e.g. polish master and hand polishing) to provide a suitable surface finish and engraved and used in conventional manner. Alternatively, and depending upon the surface finish, the printing surface may be engraved with an image for printing without machining and polishing. It has been found that the use of cold spray technology in accordance with the present invention provides a print surface having a desirable combination of surface characteristics, as is required in the printing process. In an embodiment, after engraving the printing surface may be chrome plated to provide enhanced wear characteristics.

The present invention also relates to a printing cylinder prepared in accordance with the method of the present invention, and to the use of such a cylinder in a printing process.

Embodiments of the present invention are illustrated in the following non-limiting examples.

These examples use a Kinetic 3000 cold spray system from CGT (Cold Gas Technology Grabbed which has been built based on US 5,302,414. This system consists of a LINSPRAY© gas heater, powder feeder and gun with a standard jet. CGT's long tungsten carbide nozzle was used.

### Example 1

A layer of a copper/zinc alloy (91 wt% copper and 9 wt%) was deposited on an aluminium cylinder (diameter 150 mm and length 359 mm). The powder used was a 15 - 32 micron powder with average particle size 15 micron available from ACL Bearing Company, Australia. The cylinder was rotated at a constant speed of 140 rpm and the spray gun traverse speed was 20 cm/min using the following operating parameters:

| Gas: | Nitrogen |
|---|---|
| Pressure in the heater: | 28.5 bar |
| Pressure at the jet: | 28.5 bar |
| Temperature in the heater: | 795°C |
| Temperature at the jet: | 685°C |
| Spray angle: | 90° |
| Stand off: | 25 mm |
| Feeding rate: | 2 rpm |
| Proportion of gas going to powder feeder: | 5.5% |

The thickness of the layer was 300-350 µm following by machining to provide a finished layer having a thickness of 150 -200 µm.

The average hardness of the coated layer was 280 VHN and an industry trial confirmed the suitability of the surface for engraving.

### Example 2

A layer of a copper was deposited on an aluminium cylinder (diameter 120mm and length 168 mm) rotated at a constant speed of 140 rpm and spray gun traverse speed was 20 cm/min was used. Oxygen free high conductivity (OFHC) copper powder was obtained from Metal Spray Supplies Australia with average particule size of 15 microns. The following operating parameters were used:

| | |
|---|---|
| Gas: | Nitrogen |
| Pressure in the heater: | 25 bar |
| Pressure at the jet: | 25 bar |
| Temperature in the heater: | 795°C |
| Temperature at the jet: | 700°C |
| Spray angle: | 90° |
| Stand off: | 25 mm |
| Feeding rate: | 1.8 rpm |
| Proportion of gas going to powder feeder: | 5% |

The thickness of the layer was 300-350 µm following by machining to provide a finished layer having a thickness of 150-200 µm.

The average hardness of the coated layer was 190 VHN and requires improvement to be suitable for electronic engraving.

### Example 3

A layer of zinc was deposited on an aluminium cylinder (diameter 150 mm and length 359 mm) rotated at a constant speed of 140 rpm and the spray gun traverse speed was 10 cm/min. The powder was obtained from Australian Metal Powders Supplies Pty Ltd (AMPS) and the average particle size was 15 µm. The following operating parameters:

| | |
|---|---|
| Gas: | Nitrogen |
| Pressure in the heater: | 20 bar |
| Pressure at the jet: | 20 bar |
| Temperature in the heater: | 480°C |
| Temperature at the jet: | 385°C |
| Spray angle: | 90° |
| Stand off: | 18 mm |
| Feeding rate: | 1.8 rpm |
| Proportion of gas going to powder feeder: | 16% |

The thickness of the layer was 250-300 µm following by machining to provide a finished layer having a thickness of 150-200 µm.

The average hardness of the coated layer was 108 VHN and the layer was engraved using a laser. An industry trial confirmed the suitability of the surface laser engraving.

Throughout this specification and the claims which follow, unless the context requires otherwise, the word "comprise", and variations such as "comprises" and "comprising", will be understood to imply the inclusion of a stated integer or step or group of integers or steps but not the exclusion of any other integer or step or group of integers or steps.

The reference to any prior art in this specification is not, and should not be taken as, an acknowledgment or any form of suggestion that that prior art forms part of the common general knowledge in Australia.

## Claims

1. A method of manufacturing a printing cylinder, which comprises cold-gas dynamic spraying of metal or metal alloy particles directly onto the outer surface of a substrate cylinder.

2. The method of claim 1, which comprises spraying particles of an alloy of copper and zinc.

3. The method of claim 2, wherein the alloy particles comprise 88-99 wt% copper and 12-1 wt% zinc.

4. The method of claim 3, wherein the alloy particles comprise 91 wt% copper and 9 wt% zinc.

5. The method of claim 2, wherein the average particle size of the particles is from 15 to 32µm.

6. The method of claim 2, wherein a deposited layer having a thickness of 300-350 µm is formed.

7. The method of claim 1, wherein the printing surface is formed by spraying particles of copper or an alloy of copper and zinc when the printing surface is to be subjected to electronic engraving.

8. The method of claim 7, wherein the copper has an average particle size of 10 µm.

9. The method of claim 1, wherein the metal is zinc when the printing surface is to be subjected to laser engraving or electronic engraving.

10. The method of claim 9, wherein the zinc has an average particle size of 7 µm.

11. The method of claim 1, further comprising machining and polishing the printing surface to produce a finished surface and engraving the finished surface with an image for printing, or further comprising engraving the printing surface with an image for printing.

12. The method of claim 11, further comprising chrome plating the printing surface.

13. A printing cylinder when obtained by the method of claim 1, claim 11, or claim 12.

14. Use of a printing cylinder when obtained by the method of claim 11 or claim 12 in a printing process.

## Patentansprüche

1. Verfahren zur Herstellung eines Druckzylinders, umfassend die dynamische Kaltgasbesprühung der Außenfläche eines Substratzylinders mit Metallteilchen oder Metallegierungsteilchen.

2. Verfahren nach Anspruch 1, umfassend das Aufsprühen von Teilchen einer Legierung aus Kupfer und Zink.

3. Verfahren nach Anspruch 2, bei dem die Legierungsteilchen 88 - 99 Gew.-% Kupfer und 12 - 1 Gew.-% Zink umfassen.

4. Verfahren nach Anspruch 3, bei dem die Legierungsteilchen 91 Gew.-% Kupfer und 9 Gew.-% Zink umfassen.

5. Verfahren nach Anspruch 2, bei dem die durchschnittliche Teilchengröße der Teilchen 15 µm bis 32 µm beträgt.

6. Verfahren nach Anspruch 2, bei dem eine aufgebrachte Schicht mit einer Dicke von 300 - 350 µm gebildet wird.

7. Verfahren nach Anspruch 1, bei dem die Druckfläche durch Aufsprühen von Kupferteilchen oder Teilchen einer Legierung aus Kupfer und Zink gebildet wird, wenn die Druckfläche einem elektronischen Gravurvorgang unterzogen werden soll.

8. Verfahren nach Anspruch 7, bei dem das Kupfer eine durchschnittliche Teilchengröße von 10 µm hat.

9. Verfahren nach Anspruch 1, bei dem das Metall Zink ist, wenn die Druckoberfläche einem Lasergravur- oder elektronischen Gravurvorgang unterzogen werden soll.

10. Verfahren nach Anspruch 9, bei dem das Zink eine durchschnittliche Teilchengröße von 7 µm hat.

11. Verfahren nach Anspruch 1, des Weiteren umfassend das maschinelle Bearbeiten und Polieren der Druckfläche zur Erzeugung einer fertig bearbeiteten Fläche und Eingravieren eines zu druckenden Bilds in die fertig bearbeitete Fläche, oder des Weiteren umfassend das Eingravieren eines zu druckenden Bilds in die fertig bearbeitete Oberfläche.

12. Verfahren nach Anspruch 11, des Weiteren umfassend das Verchromen der Druckfläche.

13. Druckzylinder, der gemäß dem Verfahren von Anspruch 1, Anspruch 11 oder Anspruch 12 2 hergestellt wurde.

14. Verwendung eines gemäß dem Verfahren von Anspruch 11 oder Anspruch 12 hergestellten Druckzylinders in einem Druckverfahren.

## Revendications

1. Procédé de fabrication d'un cylindre d'impression qui comprend la projection dynamique par gaz froid de particules de métal ou d'alliage de métal directement sur la surface extérieure d'un cylindre de substrat.

2. Procédé selon la revendication 1, qui comprend la projection de particules d'un alliage de cuivre et de zinc.

3. Procédé selon la revendication 2, dans lequel les particules d'alliage comprennent 88-99 % en poids de cuivre et 12-1 % en poids de zinc.

4. Procédé selon la revendication 3, dans lequel les particules d'alliage comprennent 91 % en poids de cuivre et 9 % en poids de zinc.

5. Procédé selon la revendication 2, dans lequel la taille moyenne des particules va de 15 à 32 µm.

6. Procédé selon la revendication 2, dans lequel une couche déposée de 300-350 µm d'épaisseur est formée.

7. Procédé selon la revendication 1, dans lequel la surface d'impression est formée par projection de particules de cuivre ou d'un alliage de cuivre et de zinc lorsque la surface d'impression doit être soumise à la gravure électronique.

8. Procédé selon la revendication 7, dans lequel le cuivre a une taille de particule moyenne de 10 µm.

9. Procédé selon la revendication 1, dans lequel le métal est du zinc lorsque la surface d'impression doit être soumise à la gravure au laser ou à la gravure électronique.

10. Procédé selon la revendication 9, dans lequel le zinc a une taille de particule moyenne de 7 µm.

11. Procédé selon la revendication 1, comprenant en outre l'usinage et le polissage de la surface d'impression pour produire une surface finie et la gravure d'une image d'impression sur la surface finie ou comprenant en outre la gravure d'une image d'impression sur la surface d'impression.

12. Procédé selon la revendication 11, comprenant en outre le chromage de la surface d'impression.

13. Cylindre d'impression obtenu par le procédé selon la revendication 1, la revendication 11 ou la revendication 12.

14. Utilisation d'un cylindre d'impression obtenu par le procédé selon la revendication 11 ou la revendication 12 dans un processus d'impression.
